

Nov. 15, 1949

D. DEAN ET AL  
PROCESS OF MAKING A PHOTOGRAPHIC MASK OF  
HIGH ISOELECTRIC POINT GELATIN  
Filed Feb. 28, 1948

2,487,858



DAVID DEAN  
ROBERT C. HOUCK  
INVENTORS  
*Newton M. Perris*  
BY *R. Frank Smith*  
ATTORNEYS

## UNITED STATES PATENT OFFICE

2,487,858

PROCESS OF MAKING A PHOTOGRAPHIC  
MASK OF HIGH ISOELECTRIC POINT  
GELATINDavid Dean and Robert C. Houck, Rochester,  
N. Y., assignors to Eastman Kodak Company,  
Rochester, N. Y., a corporation of New Jersey

Application February 28, 1948, Serial No. 12,017

3 Claims. (Cl. 95—2)

1

This invention relates to color photography and particularly to a method of masking or color correction for use in color photography. It is well known that the light absorptions of the dyes or coloring material used in three-color subtractive photography are incorrect in certain spectral regions. It is customary to use a mask when printing from a three-color photographic image in order to overcome the effects of the undesired spectral absorptions. The usual method of compensating for the deficiencies of the dyes or color materials in such processes consists in the use of a negative color correction mask in contact with the transparency when making the printing exposure as described, for example, in Evans U. S. Patent 2,203,653; Hanson U. S. 2,294,981 and elsewhere.

A convenient method of masking a three-color photographic transparency is described in Evans and Hanson U. S. Patent 2,371,746, granted March 20, 1945. According to the method described in that patent, a sensitive emulsion is placed in contact with the color transparency and is exposed through the transparency with light of suitable color to effect the desired correction. The film thus exposed is then removed and processed to a relief image which is dyed gray and which may be retouched with colored dyes to secure the desired correction. The relief image is applied with its support side to the emulsion of the color transparency and the combined structure may then be exposed to obtain a corrected color print. This method has the disadvantage that the masking film must be removed from the color transparency after the masking exposure in order to process the masking image. If the relief masking image were placed in a dye bath while in contact with the color transparency, the dye would contaminate the color transparency. When the masking film is removed from the color transparency, it must be re-registered with the color transparency in order to make the printing exposure.

It is therefore an object of the present invention to provide a masking method which will secure the advantages of the relief mask of Evans and Hanson U. S. Patent 2,371,746 without the attendant disadvantages. A further object of our invention is to provide a masking method in which the masking emulsion may be permanently

2

secured to the color transparency. A further object is to provide a masking emulsion which may be dyed while in contact with the usual multi-layer transparency without dyeing the multi-layer material. Other objects will appear from the following description of our invention.

These objects are accomplished according to our invention by using for the masking emulsion a gelatin having a higher isoelectric point than the gelatin used in the color transparency. This permits the masking image to be dyed without dyeing the gelatin of the color transparency, as described more fully hereinafter.

In the accompanying drawing, the figure is a flow sheet showing the film in sectional views at various stages in our process.

Our method is intended for use with all types of photographic transparencies, for example, a multi-color image produced by the process of 20 Mannes and Godowsky U. S. Patent 2,252,718, granted August 19, 1941. A multi-color transparency produced as described in that patent consists, for example, of a support having thereon superposed emulsion layers which are processed 25 to obtain cyan, magenta and yellow dye images respectively. The dyes used in such transparencies are deficient with respect to spectral absorption as mentioned above and a masking correction is desirable when printing from the 30 image in the transparency. The gelatin ordinarily used in such films is a lime-process gelatin which has an isoelectric point at approximately pH 5.

The masking film which we propose to use has 35 an emulsion made from gelatin having a higher isoelectric point than that of the gelatin used in the color transparency emulsions. It is convenient to use for the masking emulsion an acid process gelatin having an isoelectric point in the 40 region of pH 7 and upwards. Such gelatin and a method of producing it are described in Sheppard and Hudson U. S. Patent 2,101,877, granted December 14, 1937. It is well known that such 45 gelatin may be dyed with acid dyes, whereas the ordinary lime-process gelatin having an isoelectric point in the neighborhood of pH 5 would not be substantially dyed, provided that a suitable pH is chosen for the dye bath ("The Sorption of Soluble Dyes by Gelatin," Sheppard, Houck

and Dittmar, Journal of Physical Chemistry, vol. 46, 1942, page 158).

According to our process a gelatin emulsion made from high isoelectric point gelatin such as an acid-process gelatin is used as the masking material. This emulsion may be coated on the thin support of a dry-stripping material or may be of some other structure which permits its application to the color transparency to be masked. The support of the masking emulsion is cemented to the emulsion side of the multi-color transparency in any suitable way as by the use of a gelatin cement or other cement. This leaves the emulsion of the masking material outermost or away from the multi-color emulsions. An alternative method of applying the masking emulsion would be to cement the emulsion side of the masking film, as a stripping film, to the support side of the transparency. The support of the stripping film would then be removed. It will generally be desirable to use a panchromatic masking emulsion so that any of various desired corrections may be secured. Generally, it is desirable to expose the masking emulsion with red monochromatic light through the color transparency.

After exposure of the masking material through the color transparency, the entire film was placed in a developer of the following composition for 5 minutes at 68° F.

|                                  | Grams |
|----------------------------------|-------|
| Monomethyl p-aminophenol sulfate | 2.5   |
| Sodium sulfite (dessicated)      | 30    |
| Hydroquinone                     | 2.5   |
| Sodium metaborate                | 10    |
| Potassium bromide                | 0.5   |
| Water to 1 liter                 |       |

The sandwich was then washed for five minutes and treated for four minutes in the following solution in order to tan the gelatin in the region of the developed image.

*R-10 Formula (without acid)*

Stock Solution A:

|                     |       |     |
|---------------------|-------|-----|
| Water               | cc    | 500 |
| Ammonium bichromate | grams | 20  |
| Water to make       | liter | 1.0 |

Stock Solution B:

|                 |       |     |
|-----------------|-------|-----|
| Water           | liter | 1.0 |
| Sodium chloride | grams | 45  |

Add 1 part of B to 1 part of A.

After a one-minute rinse, the material was washed in water at 120° F. until clear, and the silver removed by bleaching in a ferricyanide bath of the following composition for two minutes:

|                        | Grams |
|------------------------|-------|
| Potassium ferricyanide | 80    |
| Potassium bromide      | 50    |
| Water to 1 liter       |       |

followed by treatment in a hypo solution of the following composition for 10 minutes:

|                             | Grams |
|-----------------------------|-------|
| Sodium thiosulfate          | 320   |
| Sodium sulfite (dessicated) | 10    |
| Water to 1 liter            |       |

The relief image thus formed was dyed by placing the entire sandwich in a dye solution at pH 5.5 for approximately 4 minutes to produce the desired dye density. Suitable acid dyes which may be used depending upon the correction desired are Anthraquinone Blue (C. I. 1089) and Orange II (C. I. 151) (J. S. Chem. Ind. 1887, page 591).

Both of these dyes are acid dyes and dye the gelatin of the masking image easily, without appreciably dyeing the gelatin of the color transparency.

5 Other suitable dyes, together with their Color Index numbers, are:

|                    | Color Index No. |
|--------------------|-----------------|
| Thiocarmine R      | 928             |
| Tartrazine         | 640             |
| 10 Acid green      | 670             |
| Acid violet        | 699             |
| Alizarin Rubinol R | 1091            |
| Biebrich scarlet   | 280             |
| Croceine orange    | 26              |
| 15 Lisoamine green | 737             |
| Ponceau S          | 79, 80, 252     |

The gelatin which we used for the masking emulsion had an isoelectric point at about 8.8 while the isoelectric point of the gelatin of the color transparency was about 4.8. The usual lime-process gelatin has an isoelectric point in the region of 4.7 to 5.0 and acid process gelatin ordinarily has an isoelectric point less sharply defined but in the region of pH 7 and upwards.

20 25 It is not necessary to our process that the isoelectric points be this far removed from each other. For example, differential dyeing may be secured with an acid gelatin having an isoelectric point at a pH of 6 or 7 when the pH of the isoelectric point of the gelatin of the color transparency is approximately 4.7 to 5.0. The pH of the dye bath is also a critical factor in obtaining differential dyeing as pointed out in the publication by Sheppard, Houck and Dittmar in Journal

30 35 of Physical Chemistry, referred to above. The pH of the dye bath must be above the pH of the isoelectric point of the gelatin of the color transparency and should be below the pH of the isoelectric point of the gelatin of the masking emulsion.

40 According to a modification of our invention, the masking emulsion of high isoelectric point gelatin is a stripping emulsion on a temporary support, and may be laminated either to the emulsion side or to the support side of the multi-color transparency to be masked. The support of the stripping film is removed before or after exposure of the masking emulsion, leaving the emulsion attached to the multi-color transparency. If the masking emulsion is applied to the support side of the multi-color transparency, it may be removed after printing the masked transparency, by swabbing with water.

Our invention will now be described by reference to the accompanying drawing. As shown in the first stage of the drawing, a color transparency consisting of a support 10 having thereon emulsion layers 11, 12 and 13 containing cyan, magenta and yellow images, respectively, in low isoelectric point gelatin is in contact with the masking film consisting of a transparent support 14 having thereon a sensitive silver halide emulsion 15 made from high isoelectric point gelatin. As stated above, the masking film may be laminated to the emulsion 13 in any convenient way.

65 70 After exposure of the masking emulsion through the color transparency, the masking emulsion is developed, hardened, washed off to form a relief and dyed as described above. This leaves a dyed relief gelatin mask 16 as shown in the second stage of the drawing.

According to a further modification of our invention, if the color transparency is made from gelatin having a high isoelectric point, such as acid process gelatin with an isoelectric point at

pH 6 or above, the masking emulsion may be of low isoelectric point gelatin, for example, at a pH of 4.7 to 5. In this case, a basic dye or mixture of dyes, such as Chrysoidine (Color Index, No. 21) and Methyl violet (Color Index, No. 680) may be used to dye the gelatin of the mask. Basic dyes dye gelatin only at a pH above that of its isoelectric point. The dye bath would be used at a pH between the pH's of the isoelectric points of the two types of gelatin in the transparency 10 and mask, to dye only the mask.

The term "gelatin" as used herein, includes ordinary lime-process gelatin, acid-process gelatin as defined above, gelatin derivatives and deaminated gelatin such as the gelatin described 15 in Sheppard and Hudson U. S. patent application Serial No. 631,216, filed November 27, 1945, now abandoned.

It will be understood that the examples and modifications included herein are illustrative only and that the invention is to be taken as limited only by the scope of the appended claims.

We claim:

1. A process of making a color-corrected color print which comprises laminating to a multi-color transparency having multi-colored subtractive dye images in emulsions of gelatin having an isoelectric point of about pH 4.7 to 5.0, a masking film having a single layer silver halide emulsion in gelatin having an isoelectric point of pH greater than that of the gelatin of the

transparency, exposing said masking emulsion through the color transparency and, while the masking film is in contact with the multi-color transparency, dyeing the masking emulsion with an acid dye at a pH above that of the isoelectric point of the gelatin of the color transparency and below that of the isoelectric point of the gelatin of the masking emulsion.

2. The process of claim 1 in which the gelatin of the emulsion of the masking film is an acid-process gelatin.

3. The process of claim 1 in which the gelatin of the emulsion of the masking film has an isoelectric point in the region of pH 7 and upwards.

DAVID DEAN.

ROBERT C. HOUCK.

#### REFERENCES CITED

The following references are of record in the file of this patent:

#### UNITED STATES PATENTS

| Number    | Name          | Date          |
|-----------|---------------|---------------|
| 2,266,435 | Nadeau et al. | Dec. 16, 1941 |
| 2,362,593 | Staehle       | Nov. 14, 1944 |
| 2,367,551 | Yule          | Jan. 16, 1945 |
| 2,371,746 | Evans et al.  | Mar. 20, 1945 |

#### OTHER REFERENCES

30 Journal of Physical Chemistry, vol. 46, 1942, pp. 158-176.